

## UNITED STATES PATENT OFFICE

2,507,154

DIRECT POSITIVE PHOTOGRAPHS USING  
COLOR DEVELOPERS

Dudley B. Glass and Forrest A. Richey, Rochester,  
N. Y., assignors to Eastman Kodak Company,  
Rochester, N. Y., a corporation of New Jersey.

No Drawing. Application October 17, 1947,  
Serial No. 780,574

6 Claims. (Cl. 95—5)

1

This invention relates to photography and particularly to a method of making direct positive photographs.

In Fallesen U. S. application Serial No. 780,405 filed October 17, 1947, now Patent No. 2,497,875, February 21, 1950, a method was described for making direct positive photographs which would not require solarization, a second exposure or redevelopment. According to the Fallesen application, a suitable silver halide emulsion layer, preferably an internal latent image emulsion was exposed and developed in a photographic developer capable of giving aerial fog. This method produces a positive image directly without any intermediate or additional step other than treatment in the single developing solution which gives aerial fog. The aerial fog may be produced by bubbling air through the developing solution in contact with the emulsion surface of the photograph during development or by adding agents such as certain copper salts or hydrogen peroxide to the developing solution.

We have now found that a direct positive photograph may be produced without the use of aerial fogging agents by developing the exposed special emulsion in a developing solution containing a primary aromatic amino developing agent and an active methylene coupler compound.

The photographic emulsion used in the process of our invention may be a suitable internal latent image emulsion such as a silver bromide, silver bromoiodide or silver chloroiodide emulsion. It should be undigested or, if digested, the digestion should be carried out without the use of sulfur sensitizer. A suitable emulsion is that known as Burton's emulsion described in Wall, "Photographic Emulsions," 1929, pages 52 and 53. Burton's emulsion is made as follows:

A. Silver nitrate ----- grams 100  
Water ----- cubic centimeters 500  
Ammonia—to form clear solution.  
B. Potassium bromide ----- grams 80  
Potassium iodide ----- do 50  
Soft gelatin ----- do 20  
Water ----- cubic centimeters 1000  
C. Dry gelatin ----- grams 250

B is heated to 70° C. and A, cold, added to B with constant shaking, digested for 20 minutes at 50° C., and allowed to cool slowly. C is added after being allowed to swell for 20 minutes in water, drained and melted. The emulsion is then set and washed.

An "internal latent image" emulsion, that is, one which forms the latent image mostly inside

2

the silver halide grains, as described on pages 296 and 297 of Mees "The Theory of the Photographic Process," 1942, is especially useful for the process of our invention.

Most of the "internal latent image" emulsions are silver bromo-iodide emulsions of high iodide content, preferably containing at least 10%—20% of iodide. Burton's emulsion is an emulsion of this type, having a silver iodide content of approximately 40% of the content of silver halide. Our invention is not, however, limited to the use of emulsions containing silver iodide.

An "internal latent image" made as described in Davey and Knott U. S. application Serial No. 790,232 filed December 6, 1947, now abandoned, may also be used according to our invention. This emulsion is prepared by first forming in the absence of ammonia and in one or more stages silver salt grains consisting at least partly of a silver salt which is more soluble in water than silver bromide, subsequently converting the grains to silver bromide or silver-bromo-iodide and if the silver iodide content of the emulsion is less than 6% calculated on the total silver halide, treating such grains with an iodine compound to bring the silver iodide up to at least 6%, ripening preferably in the absence of ammonia and then either washing out some of the soluble salts or washing out the whole of the soluble salts, followed by the addition of soluble salts such as soluble chloride or bromide. An example of an emulsion made in this way is as follows:

Solution No. 1:

35 Inert gelatine ----- 20 grams  
KCl ----- 20 grams } at 40° C.  
Water ----- 560 cc.

Solution No. 2:

40 KCl ----- 100 gms.  
Water ----- 520 cc. } at 45° C.

Solution No. 3:

AgNO<sub>3</sub> ----- 195 gms.  
Water ----- 520 cc. } at 45° C.

45 Solution No. 4:

KBr ----- 160 gms.  
KI ----- 40 gms. } at 45° C.  
Water ----- 500 cc.

Run solutions Nos. 2 and 3 simultaneously into 50 solution No. 1 in a vessel, taking 90 seconds to do this. Then ripen for 1 minute at 45° C. Next add solution No. 4. Then ripen for 20 minutes at 45° C. Next add 235 grams of inert gelatine (dry). Then ripen at 45° C. for 15 minutes during which time the gelatine dissolves. Set and

shred the emulsion and then wash until free from all soluble bromide and then add about 150 cc. of 10% solution of KCl (by weight), and then add water to make 3½ litres.

An "internal latent image" type of silver halide emulsion may be defined as one which, when a test portion is exposed to a light intensity scale for a fixed time between  $1/100$  and 1 second, and developed for 4 minutes at  $20^{\circ}\text{C}$ . in the ordinary, "surface" developer (Example 1), exhibits a maximum density not greater than  $1/2$  the maximum density obtained when the same emulsion is equally exposed and developed for 3 minutes at  $20^{\circ}\text{C}$ . in an "internal" type developer. Stated conversely, an "internal latent image" emulsion, when developed in an "internal" type developer (Example 2) exhibits a maximum density at least 5, and preferably at least 10, times the maximum density obtained when the same emulsion is exposed in the same way and developed in a "surface" developer (Example 1).

Our process depends on the use, with the internal latent image emulsion, of a developing solution containing an active methylene compound, a primary aromatic amino developing agent, little or no anti-foggant and no active silver halide solvent such as sodium thiosulfate or sodium thiocyanate. When these conditions are satisfied, immersion of the exposed emulsion in the developing solution yields a direct positive image at the same sensitometric speed as the negative speed of the emulsion.

The aromatic amino developing agent used in the developing solution may comprise any of the suitable aromatic amino developing agents normally used in color photographic processes such as the p-phenylenediamines and p-aminophenols. Derivatives of these developers formed by substitution in the amino group as well as in the ring such as the alkyl phenylene diamines and alkyl toluylene diamines may also be used. Suitable compounds as diethyl-p-phenylenediamine hydrochloride, monomethyl-p-phenylenediamine hydrochloride, dimethyl-p-phenylenediamine sulfate, 2-amino-5-ethylaminotoluene hydrochloride and the developing agents described in Weissberger U. S. Patent 2,193,015.

The active methylene compounds used in the developing solution are those which are normally used in color photography and contain a reactive methylene group of the following type:



Couplers of the phenolic hydroxyl type are not suitable for use according to our invention.

The following coupler compounds are suitable as the active methylene compound for incorporation in the developing solution: acetoacetanilide, 2,5-dichloro-acetoacetanilide, omega-benzoyl-acetanilide, omega-benzoyl-4-(p-tolylsulfonamido)-acetanilide, 2-cyanoacetylcoumarone, 3-(m-nitrobenzamido)-1-phenyl-5-pyrazolone and other compounds described in U. S. Patents 2,108,602, 2,271,238 and 2,369,489.

The developing solution should contain little or no anti-foggant. The use of certain anti-foggants not containing labile sulfur such as benzotriazole may be tolerated but such compounds do not aid in obtaining the direct positive action.

The developer should have a low sulfite content and should not contain any active silver halide solvent such as sodium thiosulfate or sodium thiocyanate. No silver halide solvent more powerful (as a silver halide solvent) than sulfite should be used.

An ordinary "surface type" developer, that is, one which develops an image only on the surface of the grains of an "internal latent image" emulsion is the following:

*Example 1*

|                             | Grams |
|-----------------------------|-------|
| p-Hydroxyphenylglycine      | 10    |
| Sodium carbonate (crystals) | 100   |
| Water to 1 liter.           |       |

Development time, 4 min. at  $20^{\circ}\text{C}$ .

An "internal type" developer, that is, one which develops an image inside the grains of an "internal latent image" emulsion, is the following:

*Example 2*

|                                     | Grams |
|-------------------------------------|-------|
| Hydroquinone                        | 15    |
| 25 Monomethyl-p-aminophenol sulfate | 15    |
| Sodium sulfite (anhydrous)          | 50    |
| Potassium bromide                   | 10    |
| Sodium hydroxide                    | 25    |
| Sodium thiosulfate (crystals)       | 20    |
| 30 Water to 1 liter.                |       |

Development time, 3 min. at  $20^{\circ}\text{C}$ .

Our invention will now be described by reference to the following specific example.

An emulsion such as that described in the Davey and Knott U. S. application Serial No. 790,232 described above was coated on a support, dried and exposed on an Eastman 2B Sensitometer (Journal Society Motion Picture Engineers, vol. 17, 1931, page 536). The exposed emulsion was then developed 15 minutes at  $65^{\circ}\text{F}$ . in the following developing solution:

*Example 3*

|                                                  | Grams |
|--------------------------------------------------|-------|
| 45 2-amino-5-diethyl-amino-toluene hydrochloride | 3     |
| Sodium sulfite                                   | 5     |
| Sodium carbonate                                 | 20    |
| Sodium hydroxide                                 | 1     |
| 50 2,5-dichloro-acetoacetanilide                 | 3     |
| Water to 1 liter.                                |       |

The emulsion was then fixed in hypo and washed. The image produced in this way was a dye image containing metallic silver. The silver can be removed with ferricyanide and hypo to leave a pure yellow dye image in the layer.

An alternative procedure involves the use of a two-bath development step as described in Ives U. S. application Serial No. 780,318 filed October 17, 1947. According to this method, the exposed emulsion layer of the internal latent image type is immersed for thirty seconds in the following solution:

*Example 4*

|                                               | Grams |
|-----------------------------------------------|-------|
| 2-amino-5-diethyl amino toluene hydrochloride | 3     |
| Sodium sulfite (dessicated)                   | 3     |
| Sodium carbonate monohydrate                  | 30    |
| Sodium hydroxide                              | 3     |
| 70 Acetoacet-2,5-dichloroanilide              | 3     |

When the exposed emulsion is immersed in this solution for only 30 seconds, no visible image is produced but a positive silver image is obtained

when the emulsion is then immersed for 1 to 1½ minutes in a developer of the following composition:

*Example 5*

|                                   | Grams |
|-----------------------------------|-------|
| Hydroquinone -----                | 45    |
| Sodium sulfite (dessicated) ----- | 90    |
| Sodium hydroxide -----            | 38    |
| Potassium bromide -----           | 30    |
| Water to 1 liter.                 |       |

The developer of Example 5 is an active developer and by the use of the developers of Example 4 and Example 5, an image is produced in 1 to 2 minutes as compared with a time of five or six minutes if the film is allowed to remain in the developer of Example 3 or Example 4 for the entire development time.

It will be evident to those skilled in the art that our process affords a convenient means for obtaining a direct positive photograph either in color or in metallic silver by simple exposure and development steps and avoids the necessity of high intensity exposures or a second exposure or re-development. It will be understood that the examples and modifications included herein are illustrative only and that their invention is to be taken as limited only by the scope of the appended claims.

We claim:

1. The method of obtaining a direct positive dye image in a silver halide emulsion layer, which comprises exposing to light rays to which the emulsion is sensitive, a silver halide emulsion layer, a test portion of which upon exposure to a light intensity scale for a fixed time between  $1/100$  and 1 second and development for 3 minutes at 20° C. in the following internal type developer (II):

|                                        | Grams |
|----------------------------------------|-------|
| Hydroquinone -----                     | 15    |
| Monomethyl-p-aminophenol sulfate ----- | 15    |
| Anhydrous sodium sulfite -----         | 50    |
| Potassium bromide -----                | 10    |
| Sodium hydroxide -----                 | 25    |
| Sodium thiosulfate -----               | 20    |
| Water to 1 liter.                      |       |

gives a maximum density at least 5 times the maximum density obtained when the equally exposed silver halide emulsion is developed for 4 minutes at 20° C. in the following surface developer (I):

|                              | Grams |
|------------------------------|-------|
| p-Hydroxyphenylglycine ----- | 10    |
| Sodium carbonate -----       | 100   |
| Water to 1 liter.            |       |

and immediately immersing said layer in a single developing solution free of anti-fogging containing labile sulfur and free of silver halide solvent more powerful as a silver halide solvent than sulfite and containing a primary aromatic amino developing agent and an active methylene coupler compound capable of coupling with the oxidation product of said developing agent to produce a dye image in said solution, for a length of time sufficient to produce a positive dye image in said layer.

2. The method of obtaining a direct positive image in a silver halide emulsion layer, which comprises exposing to light rays to which the emulsion is sensitive, a silver halide emulsion layer, a test portion of which upon exposure to a light intensity scale for a fixed time between  $1/100$  and 1 second and development for 3 minutes at

20° C. in the following internal type developer (II):

|                                        | Grams |
|----------------------------------------|-------|
| Hydroquinone -----                     | 15    |
| Monomethyl-p-aminophenol sulfate ----- | 45    |
| Anhydrous sodium sulfite -----         | 50    |
| Potassium bromide -----                | 10    |
| Sodium hydroxide -----                 | 25    |
| Sodium thiosulfate -----               | 20    |
| Water to 1 liter.                      |       |

gives a maximum density at least 5 times the maximum density obtained when the equally exposed silver halide emulsion is developed for 4 minutes at 20° C. in the following surface developer (I):

|                              | Grams |
|------------------------------|-------|
| p-Hydroxyphenylglycine ----- | 10    |
| Sodium carbonate -----       | 100   |
| Water to 1 liter.            |       |

and then without intermediate treatment, rendering developable the silver halide grains in the unexposed regions of said layer by immersing said layer in a developing solution free of anti-fogging containing labile sulfur and free of silver halide solvent more powerful as a silver halide solvent than sulfite and containing a primary aromatic amino developing agent and an active methylene coupler compound capable of coupling with the oxidation product of said developing agent to produce a dye image, and developing to metallic silver said grains thus rendered developable.

3. The method of obtaining a direct positive image in a silver halide emulsion layer, which comprises exposing to light rays to which the emulsion is sensitive, a silver halide emulsion layer, a test portion of which upon exposure to a light intensity scale for a fixed time between  $1/100$  and 1 second and development for 3 minutes at 20° C. in the following internal type developer (II):

|                                        | Grams |
|----------------------------------------|-------|
| Hydroquinone -----                     | 15    |
| Monomethyl-p-aminophenol sulfate ----- | 15    |
| Anhydrous sodium sulfite -----         | 50    |
| Potassium bromide -----                | 10    |
| Sodium hydroxide -----                 | 25    |
| Sodium thiosulfate -----               | 20    |
| Water to 1 liter.                      |       |

gives a maximum density at least 5 times the maximum density obtained when the equally exposed silver halide emulsion is developed for 4 minutes at 20° C. in the following surface developer (I):

|                              | Grams |
|------------------------------|-------|
| p-Hydroxyphenylglycine ----- | 10    |
| Sodium carbonate -----       | 100   |
| Water to 1 liter.            |       |

and then without intermediate treatment, rendering developable the silver halide grains in the unexposed regions of said layer by immersing said layer in a developing solution free of anti-fogging containing labile sulfur and free of silver halide solvent more powerful as a silver halide solvent than sulfite and containing a primary aromatic amino developing agent and an active methylene coupler compound capable of coupling with the oxidation product of said developing agent to produce a dye image, and developing to metallic silver said grains thus rendered developable.

4. The method of obtaining a direct positive image in a silver halide emulsion layer, which comprises exposing to light rays to which the emulsion is sensitive, a silver halide emulsion

75

layer, a test portion of which upon exposure to a light intensity scale for a fixed time between  $1/100$  and 1 second and development for 3 minutes at  $20^{\circ}\text{C}$ . in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at  $20^{\circ}\text{C}$ . in the following surface developer (I):

|                        | Grams |
|------------------------|-------|
| p-Hydroxyphenylglycine | 10    |
| Sodium carbonate       | 100   |
| Water to 1 liter.      |       |

and then without intermediate treatment, rendering developable the silver halide grains in the unexposed regions of said layer by immersing said layer in a developing solution free of anti-foggant containing labile sulfur and free of silver halide solvent more powerful as a silver halide solvent than sulfite and containing 2-amino-5-diethylamino toluene hydrochloride as the developing agent and an acetoacetanilide coupler compound capable of coupling with the oxidation product of said developing agent to produce a dye image, and developing to metallic silver said grains thus rendered developable.

5. The method of obtaining a direct positive image in a silver halide emulsion layer, which comprises exposing to light rays to which the emulsion is sensitive, a silver halide emulsion layer, a test portion of which upon exposure to a light intensity scale for a fixed time between  $1/100$  and 1 second and development for 3 minutes at  $20^{\circ}\text{C}$ . in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at  $20^{\circ}\text{C}$ . in the following surface developer (I):

|                        | Grams |
|------------------------|-------|
| p-Hydroxyphenylglycine | 10    |
| Sodium carbonate       | 100   |
| Water to 1 liter.      |       |

and then without intermediate treatment, rendering developable the silver halide grains in the unexposed regions of said layer by immersing said layer in a developing solution free of anti-

foggant containing labile sulfur and free of silver halide solvent more powerful as a silver halide solvent than sulfite and containing 2-amino-5-diethylamino toluene hydrochloride as the developing agent and 2,5-dichloroacetoacetanilide, and developing to metallic silver said grains thus rendered developable.

6. The method of obtaining a direct positive image in a silver halide emulsion layer, which comprises exposing to light rays to which the emulsion is sensitive, a layer of silver halide emulsion in which at least 6% of the silver halide is silver iodide, a test portion of which upon exposure to a light intensity scale for a fixed time between  $1/100$  and 1 second and development for 3 minutes at  $20^{\circ}\text{C}$ . in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at  $20^{\circ}\text{C}$ . in the following surface developer (I):

|                        | Grams |
|------------------------|-------|
| p-Hydroxyphenylglycine | 10    |
| Sodium carbonate       | 100   |
| Water to 1 liter.      |       |

35 and then without intermediate treatment, rendering developable the silver halide grains in the unexposed regions of said layer by immersing said layer in a developing solution free of anti-foggant containing labile sulfur and free of silver halide solvent than sulfite and containing a primary aromatic amino developing agent and an active methylene coupler compound capable of coupling with the oxidation product of said developing agent to produce a dye image, and developing to metallic silver said grains thus rendered developable.

DUDLEY B. GLASS.  
FORREST A. RICHEY.

#### REFERENCES CITED

The following references are of record in the file of this patent:

|                  | UNITED STATES PATENTS |               |              |
|------------------|-----------------------|---------------|--------------|
| 55               | Number                | Name          | Date         |
|                  | 2,401,051             | Crouse et al. | May 28, 1946 |
| FOREIGN PATENTS  |                       |               |              |
| 60               | Number                | Country       | Date         |
|                  | 451,347               | Great Britain | Aug. 4, 1936 |
| OTHER REFERENCES |                       |               |              |

65 Wall: "Photographic Emulsions," Publ. 1929 by Amer. Phot. Publ. Co., Boston, pages 52 and 53.